

Aug. 13, 1940.

A. N. SACHANEN ET AL

2,211,732

MOTOR FUEL

Filed Feb. 10, 1939



ALEXANDER N. SACHANEN  
ALFRED W. FRANCIS  
INVENTORS

BY  
Raymond B. Buhard  
ATTORNEY

## UNITED STATES PATENT OFFICE

2,211,732

## MOTOR FUEL

Alexander N. Sachanen and Alfred W. Francis,  
Woodbury, N. J., assignors to Socony-Vacuum  
Oil Company, Incorporated, New York, N. Y.,  
a corporation of New York

Application February 10, 1939, Serial No. 255,602

3 Claims. (Cl. 44—9)

This invention is directed to the production of motor fuel for high compression internal combustion engines, particularly aviation fuels. It is particularly directed to the provision of motor fuels combining the properties of high inherent anti-knock quality, high susceptibility to improvement of anti-knock quality by the addition of tetra-ethyl lead, and having balanced distillation characteristics suitable for proper utilization in high efficiency engines.

As is well known, the addition of aromatic compounds, such as benzene and alkylated benzenes, to gasoline, increases the anti-knock capability of the mixed fuel. There have been many proposed methods for the production of alkylated benzenes. For example, vaporous products of cracking, including olefines, in admixture with benzene, may be reacted under catalytic conditions to produce alkylated benzenes in admixture with the normally produced gasoline constituents. Benzene or certain alkyl benzenes may be reacted in the presence of aluminum chloride with olefines to form mixtures of alkylated benzenes. Benzene and olefines may be reacted at high temperatures without catalyst, with or without high pressure, or under slightly lower temperatures in the presence of catalysts such as adsorptive contact masses, to give mixtures of alkylated benzenes. Where the process is one of treatment of a mixture of gasoline and benzene, the resulting product is a mixture of gasoline and various alkyl benzenes not capable of separation by distillation. In this mixture there are present not only all of the higher boiling fractions of the gasoline but also the various alkyl benzenes which boil in the same boiling range as the higher boiling fractions of the gasoline. As will be pointed out later, such mixtures are undesirable. When the process is conducted solely for the production of alkyl benzenes as in the later examples noted above, there is produced a mixture of alkyl benzenes boiling in the same boiling range as the higher boiling constituent of gasoline. When the products of such processes are mixed with ordinary gasoline, there are present in the final mixture both the higher boiling constituents of gasoline and the alkyl benzenes which boil in the same range of temperature.

Such mixtures are not desirable for several reasons. For one thing, to insure proper carburetion and combustion of motor fuel, it is well known that the distribution of products in this boiling range should be uniform. A preponderance of either light or heavy material leads to

uneven carburetion and to uneven burning. This is recognized by users and the requirement is reflected in specifications which require reasonable distribution of material across the entire boiling range of the fuel. This is usually arrived at by specifying that some given percent of distillate shall be recovered at "not more than 5 ° F." for several points in the boiling range. A typical distillation specification for a gasoline for aviation engine use is as follows:

*Distillation characteristics*

| Percent recovered in receiver | °F. maximum  | 15 |
|-------------------------------|--------------|----|
| 5%                            | 150.         |    |
| 10%                           | 167.         |    |
| 50%                           | 212.         |    |
| 90%                           | 266.         |    |
| 96%                           | 311.         |    |
| Percent recovered             | 96% minimum. |    |
| Percent loss                  | 2% maximum.  | 20 |
| Percent residue               | 2% maximum.  |    |

This is the distillation range specification adopted for a number of fuels of varying octane number by American Airlines, as shown by 25 Table I—Domestic (U. S.) Aircraft Fuel Specifications—in "Aircraft-Fuel Specifications, Present and Future" by Hubner, Egloff and Murphy, National Petroleum News, July 28, 1937.

The real requirement of such specifications 30 may be noted by reference to the drawing attached to this specification, wherein curve 1 shows such a specification and curves 2, 3, 4, 5 show various fuels later described. The important feature of the specification, as shown by curve 35 1, is the relative amounts of low boiling and high boiling constituents, as shown by its gradual rise or slope. This specification is typical only and other fuels may vary from this in degree or slightly in kind. For example, a lighter fuel 40 of the same kind would be shown by displacing curve 1 downwardly without change of slope, or a heavier one by displacing curve 1 upwardly. To specify fuels somewhat higher in light constituents, as may be preferred by some for aviation purposes, the curve 1 could be changed somewhat in slope, falling a little lower at the low boiling end and rising a little higher on the high boiling end, yet without material increase in end point.

In contrast with curve 1, curve 2 shows an exceedingly poor fuel. This fuel is entirely too high in boiling range and not sufficiently rich in low boiling material. This curve represents the distillation range of a mixture of alkyl 55

benzenes such as may be produced by the processes hereinbefore described.

Curve 3 shows an equally poor fuel, entirely too rich in light material, although some of its heavy material is relatively high boiling. This is a commercial casinghead gasoline of 320° F. end point.

Curve 4 shows what may be achieved by a blend of equal proportions of the fuel of curve 2 and 10 the fuel of curve 3. The resulting blend, although it possesses a low initial boiling point, is entirely deficient because it has too much high boiling point material resulting from the simultaneous presence of the heavy constituents of both fuels. 15 Blending in various proportions other than 50-50 will not serve to remedy this. The fuel may be highly antiknock, but will be carbureted so poorly and unevenly that this property cannot be made use of. Fuels arising from the simultaneous 20 production of gasoline and alkyl benzenes will have similar characteristics for the same reasons.

However, if we take from the fuel of curve 2 only those portions of boiling range within that of the desired fuel, discarding the remainder, and 25 take from the fuel of curve 3 only those portions of boiling range below the selected portion of the fuel of curve 2, discarding the remainder, we may blend the two selected fractions to give a fuel having proper boiling characteristics. For example, curve 5 shows a blend of 50 per cent of 30 casinghead gasoline comprising that fraction of the fuel of curve 3 boiling below 210° F., and 50 per cent of alkyl benzenes which are the portion of the fuel of curve 2 boiling up to 300° F. Note 35 that the curve 5 is regular in form, and that because there is substantially no overlap in the boiling range of the constituents, it can be shifted in slope by changes in proportion of those constituents. 40 Of particular interest are some other properties of blends made of fuel constituents of selected properties as disclosed herein.

#### Acid heat test

45 Specification \_\_\_\_\_ Shall be not more than 20° F.  
Fuel of curve 5 \_\_\_\_\_ 7° F.

The acid heat test is based on the heat generated by shaking a specified amount of fuel with C. P. sulphuric acid of 1.83/1.84 specific gravity 50 and is a measure of undesirable and unstable (unsaturated), material present.

#### Lead susceptibility

55 Motor method octane number  
Fuel of curve 5, 85.1; fuel+3 cc. lead, 96.8; increase, 11.7

The novel blend is thus seen to retain a high lead susceptibility, a feature which has not here-

tofore been thought possible for high octane number aromatic blends containing as much as 50% aromatic hydrocarbons.

Within the limits herein taught, this disclosure may be applied to the blending of alkyl benzenes with gasoline of any origin, be it casinghead, straight run, or cracked. The method is particularly valuable when utilized for the production of aviation gasoline of unusually high quality from vapor phase catalytically cracked gasoline. 10 With a material of this type, particularly with a material such as that produced by the so-called Houdry process, wherein gas oil is catalytically cracked at temperatures of about 875° F. in the presence of a granular catalyst composed essentially of alumina and silica, aviation gasolines may be produced having nearly 100 octane value by the motor method, by the addition of a comparatively small amount of lead fluid to a properly produced blend of cracked gasoline and alkyl 15 benzenes. 20

Particularly desirable aviation fuels may be made by taking the portion of such catalytically cracked gasoline boiling below about 220° F. and blending with it a mixture of alkyl benzenes having an end point somewhat lower than that of the desired aviation gasoline, for example about 300° F. 25

We claim:

1. A motor fuel having distillation characteristics of an aviation gasoline and a smooth boiling range comprising a mixture of alkyl benzenes boiling above about 220° F. and a gasoline fraction boiling below about 220° F. 30

2. An aviation motor fuel characterized by high anti-knock value, high lead susceptibility, and balanced distillation range characteristics comprising a blend of two ingredients, one of which is a mixture of alkylated benzenes, the other of which is a low boiling material of petroleum origin substantially all of which has a boiling range 40 below that of the alkylated benzene mixture.

3. A motor fuel characterized by high inherent anti-knock value, balanced distillation range and high lead susceptibility comprising a blend of two ingredients, one of which is a mixture of alkylated benzenes having a boiling range terminating at approximately the end point of an aviation fuel, the remainder being the portion boiling below about 220° F. of a cracked gasoline produced 45 by subjecting gas oil to catalytic cracking at a temperature of about 875° F. in the presence of a catalytic contact mass composed essentially of alumina and silica.

ALEXANDER N. SACHANEN.  
ALFRED W. FRANCIS.